

Patented Sept. 11, 1928.

1,683,849

# UNITED STATES PATENT OFFICE.

HARRY MORTIMER SPECHT, OF PELHAM, NEW YORK.

## PROCESS OF IMPREGNATING FABRIC WITH SUBSTANTIALLY PERMANENT FRAGRANCE AND THE PRODUCT.

No Drawing.

Application filed September 1, 1925. Serial No. 53,957.

My invention relates to an improvement in a process of impregnating a fabric with a substantially permanent fragrance and the product produced thereby as will be more fully hereinafter pointed out.

In the present age of the very general use of face powders, the powder puff has become an article of every day use by the majority of women.

Such powder puffs are used so frequently that many women carry them with them at all times. It therefore has become important that the powder puff itself shall carry a pleasing odor or fragrance so that its use will not only not be offensive, but will be pleasing to those around whom the puff is used. A puff carrying such a desirable fragrance also will add to the desirable fragrance of the powder as used, thereby making the use of the powder more effective.

Because of the difficulty in securing a fragrance which is substantially permanent no such powder puff nor the fabric for making the same has been produced heretofore.

My process is adapted to solve this problem in that it prepares a pile fabric or the like with a substantially permanent back coating of required fragrance together with a pile or face fabric impregnation of a more volatile fragrance blending with the fragrance of the back coating without interfering with the effectiveness of the face or pile, whereby a powder puff or other article may be made of this material so treated with the assurance that it will sustain the desired pleasing fragrance as long as the same may be useful.

There are many fragrant gums which may be used to form a compound solution suitable for coating the back of a fabric but in order that we may have these definitely before us the following fragrant gums, balsams and natural and synthetic derivatives are named, all of which are suitable for the purpose, and all of which have a natural fragrance and which, in combination, will form the desired substantially permanent fragrance for our fabric. Among others we name: benzoin, labdanum, styrax, tolu, balsam peru, civet, tonkin musk, ambrette, olivebanum, guajaic wood (concrete form), oris root (concrete form) and phenyl acetic acid.

As these are all fragrant gums, balsams or natural or synthetic derivatives, a composition of all or any of them, put into so-

lution of alcohol in the usual well known manner, will, when used for coating the back of the pile fabric, form thereon not only a substantially permanent fragrant coating but one that is so soft and pliable that it can not in any way injure the softness and flexibility of the fabric, which function is highly important in the use of the fabric in a powder puff.

As powder puffs, to conform to the regular practice, must be made from a pile of fabric, it is necessary in handling such fabric to keep the pile free from any pressing or rubbing, as this tends to mat the pile and thereby spoil the desired effect and function of the pile as it is this soft, flexible and brush-like pile which picks up the powder and applies it to the face so efficiently.

Therefore, in order to dry the solution of the fragrant gum compound, it is necessary to make use of well known drying frames which are commonly used in the handling of pile fabrics whereby the fabric is held on the selvage edges in such a manner that nothing will contact with the face or pile of the fabric. These frames or racks are known as pin hook steel racks being commonly used in the handling of pile fabrics to prevent the crushing of the pile.

In order to effect the drying of the coating on the back of the fabric, the coated fabric mounted on such pin hook steel racks as described, can be placed in a steam heated vacuum retort which may be hermetically sealed and a vacuum created in said retort by means of a pump, following which the steam can be turned on to the jacketed retort permitting the fabric to remain in this vacuum under heat for a sufficient length of time to insure thorough drying of the back coating and the elimination of any other moisture in the fabric. Any other well known means which will effect the thorough drying of the back coating will answer the requirements of the process.

Making use of the retort and the vacuum therein, the fabric may be further impregnated with a volatile fragrant material combined with some of the aforementioned fragrant solution which will particularly impregnate the pile or face of the fabric by supplying an odorant having a volatile fragrance combined with the substantially permanent fragrance to the vacuum retort thereby insuring thorough impregnation of

the residue of the fabric without the loss of any substantial amount of odorant used. Such an odorant solution of volatile fragrance combined with the substantially permanent fragrant solution may also be sprayed upon the face or pile of the fabric in any well known manner without the use of any vacuum retort while the fabric is still warm from its drying whereby it will readily absorb such odorant in a more complete manner than would be possible if sprayed on to the fabric when the fabric is cold. Such impregnating or spraying of the face or pile will not in any way change the effectiveness of the pile for such use for example as required in a powder puff.

In carrying out my process a piece or length of pile fabric is first coated on the back of said fabric with a substantially permanent fragrant odor by means of the application to the back of said fabric of a solution of a compound of suitable fragrant gums, balsams or natural or synthetic derivatives. The coated pile fabric is then dried in such a manner as to dry said back coating and also eliminate any other moisture in said fabric and doing so without crushing the pile of said fabric. The dried and back coated fabric is then submitted to a further impregnation of a solution of a volatile fragrant odorant combined with a compound solution of suitable fragrant gums said combination having a fragrance adapted to blend with the fragrance of said back coating whereby said pile fabric is thoroughly impregnated with a substantially permanent fragrant odor and also impregnated with a volatile fragrant odor adapted to blend with and strengthen said permanent fragrant odor.

The fragrant gums, balsams and natural and synthetic derivatives and volatile fragrance material used in combination in the face or pile impregnation form a mixture which can only be segregated into organic and inorganic groups.

I claim:

1. The process of impregnating a fabric with a substantially permanent fragrant odor comprising coating the back of said fabric with a solution of a compound of suitable fragrant gums, drying said solution and further impregnating the face of said fabric with a combined solution of volatile and substantially permanent fra-

grant odorant adapted to blend with the fragrance of said back coating.

2. The process of impregnating a fabric with a substantially permanent fragrant odor comprising coating the back of said fabric with a solution of a compound of suitable fragrant balsams, drying said solution and further impregnating the face of said fabric with a combined solution of volatile and substantially permanent fragrant odorant adapted to blend with the fragrance of said back coating while the fabric is warm from the drying.

3. The process of impregnating a fabric with a substantially permanent fragrant odor comprising coating the back of said fabric with a solution of a compound of suitable fragrant derivatives of gums, drying said solution and further impregnating the face of said fabric with a combined solution of volatile and substantially permanent fragrant odorant adapted to blend with the fragrance of said back coating.

4. The process of impregnating a fabric with a substantially permanent fragrant odor comprising coating the back of said fabric with a solution of a compound of suitable fragrant derivatives of balsams, drying said solution and further impregnating the face of said fabric with a combined solution of volatile and substantially permanent fragrant odorant adapted to blend with the fragrance of said back coating.

5. The process of impregnating a pile fabric with a substantially permanent fragrant odor comprising coating the back of said fabric with a solution of a compound of suitable fragrant gums, drying said solution and further impregnating the face of said fabric with a combined solution of volatile and substantially permanent fragrant odorant adapted to blend with the fragrance of said back coating while the fabric is warm from the drying.

6. A new article of manufacture consisting of a pile fabric having a flexible gum coating on the back of a substantially permanent fragrance and an impregnation of the pile with a volatile and substantially permanent fragrance adapted to blend with that of the back coating.

In testimony whereof I affix my signature.

HARRY MORTIMER SPECHT.